

## UNITED STATES PATENT OFFICE.

JOHN B. AUSTIN, OF CLEVELAND, OHIO.

## PROCESS OF UNITING METALS.

No Drawing.

Application filed January 2, 1923. Serial No. 610,347.

*To all whom it may concern:*

Be it known that I, JOHN B. AUSTIN, a citizen of the United States, residing at Cleveland, in the county of Cuyahoga and

5 State of Ohio, have invented a certain new and useful Improvement in Processes of Uniting Metals, of which the following is a specification.

This invention relates to the art of uniting metals or metallic articles and especially to the uniting of copper to steel. It relates to the process of integrally uniting metals or metallic articles with what is believed to be an alloyed junction therebetween.

It also relates to the process of removing oxides from molten copper and the formation of dense substantially non-porous metal when solidified.

20 It further relates to the process of removing any oxide films which may be formed on the surface of the metal or metals to be joined together. It also relates to the thorough dissemination throughout the

25 molten metal of a suitable reagent, such as silicon, under such conditions that the reagent comes in contact with all oxide material and gases in the metal and also with any oxide on the contacting surface or sur-

30 faces of the metals to be joined and permits the union of the metals to take place throughout clean nonoxidized metallic surfaces, substantially in the absence of gases and of an oxidizing atmosphere.

35 Broadly considered my process consists in melting one metal so as to form a bath thereof in contact with another metal and disseminating throughout the bath of molten metal a quantity of a reagent cap-

40 pable of removing combined oxides from the molten bath and either removing occluded gases therefrom or retaining them in solution after solidification of the metal and also to remove any surface oxide from the

45 other metal. The molten bath is maintained at a temperature sufficiently high and for a period of time sufficiently long to cause what is believed to be a thin alloy film to form between the contacting surfaces of

50 the two metals, and/or a penetration of either or both of the metals into each other.

Although I believe the connection formed between the two metals by my process to be in the nature of an alloy or a thin alloy film, it may be a mutual inter-penetrations of the metals. Accordingly I desire to be

understood, whenever I use the terms "alloy," "alloy film," "alloy junction" or similar expressions herein, as referring to the junction formed between the two metals, whatever its exact character and structure may be provided it is similar to that formed by my process.

The reagent may be added in various ways preferably by being first incorporated in an ingot of metal which is drawn into a rod or wire and then added to the molten bath. Or it may be added as a powder or incorporated as a constituent of the metallic article to be melted or the mold employed to hold the molten metal or added in any suitable manner. This reagent which is added to the bath is thoroughly disseminated, preferably by being continuously introduced in relatively small quantities so that the bath is built up by a succession of layers or additions which are successively heated until any occluded gases have been removed or rendered harmless and the oxide destroyed. This may be accomplished by causing the heating flame to play upon the surface of the bath as the surfaces are cleaned and the desired temperature attained, the alloying of the articles taking place between clean nonoxidized surfaces, thus uniting the metals out of contact with the atmosphere or any gases and without substantially any intervening oxide. This alloying reaction is usually indicated by the formation of a concave surface of the copper bath at the point where it contacts with the iron.

By the term "reagent" as employed in this application I mean any substance, element, compound or mixture as metallic silicon possessing the property of—

(1) Reacting with occluded gases in the molten metal bath to permit their escape or to render them harmless by retaining them in solution in the metal as it solidifies,

(2) Reacting with any oxides in a molten bath to alter the form of the oxide and remove it,

(3) Reacting with any oxide on the surface of a metal in contact with such a bath to alter the oxide and remove it, and

(4) Reacting with any gases in the molten metal adjacent the surface thereof to permit their escape or to render them harmless by retaining them in solution in the metal as it solidifies.

The exact temperature of the metal form-

ing the molten bath at the time the alloying takes place is not definitely known but in the case of copper various pyrometric tests indicate that it is above the melting point of copper and below the melting point of eutectoid steel.

Describing now my improved process, more particularly for the joining of copper to steel, it consists in placing the metals 10 in surface contact. The copper may be held in any suitable manner, for example by locating the portions thereof in contact with the steel in a carbon mold which will retain heat, and which may be of any well known 15 construction. A portion of the copper is melted in the mold cavity and a predetermined quantity of a reagent such as silicon is added thereto in a suitable manner, for example, from a copper rod containing from 20 about .2% to about .3% silicon. The heat for effecting the melting may be applied by various means, such for example as an electric arc, a suitable gas flame or other heating medium, it only being necessary that 25 such medium be capable of heating the article and molten metal to the desired temperature above the melting point of copper. A portion of this rod is melted by the heating flame until it enters and commingles 30 with the molten bath and the bath is heated until the molten metal becomes fluid, as compared with copper at a temperature just above the melting point thereof, and the molten metal melts the steel as indicated by 35 a ripple like movement which takes place on the surface with the formation of a concave surface resembling a meniscus adjacent the steel. These changes indicate the completion of the reactions and the uniting 40 of the metals. Additional portions of the copper are then melted and silicon is added thereto until the occluded gases and oxides are either removed or rendered harmless, as 45 the case may be, and the alloying takes place, as indicated by the formation of the meniscus. This operation is repeated until the body of copper has been melted and what is believed to be an alloy film has 50 been formed between the contacting surfaces of the metals. It will be observed that the alloying or uniting of the metals takes place while one metal is molten and in contact with the other and after substantially all gases, slag formations and 55 oxides have been removed from between the metals and from within the molten metal. The alloying or uniting thus is effected between clean metal surfaces in the absence of gases or an oxidizing atmosphere, permitting interpenetration of the clean metals under most advantageous circumstances. In this case it is desired not to melt any appreciable amount of the steel 60 and preferably the steel is not affected in any deleterious way, and only its surface

portion unites with the copper. I have found in commercial practice that this desired melting may be obtained efficiently and economically by the use of a carbon arc. This arc may be played upon the copper so as to melt not only a portion of the copper to be joined to the steel but also the copper rod containing the reagent, and this melting may be and preferably is effected without causing the flame of the arc to come in contact with the steel. Further, I have found that the heating also may be accomplished efficiently and economically by using the copper rod containing the reagent as one electrode of a metallic arc, the work constituting the other electrode. Here again the heating may be effected without applying the flame of the metallic arc to the steel, confining it merely to the copper in its solid and molten state. In fact, where either the carbon arc or metallic arc is used as I have just mentioned, the arc may be directed upon the copper in such manner as to create a molten bath which may be maintained molten by directing the arc against it until the desired reactions have taken place and to the naked eye the molten metal in the bath appears quiet and free from the effects of escaping gases. It will be understood that when the arc is directed upon the surface of the molten metal the well known force of the arc agitates the molten metal thereby undoubtedly assisting or facilitating the thorough dissemination of the reagent throughout the molten metal and expediting the desired reactions of the reagent. In the same manner any suitable heating flame other than an electric arc, for example a gas flame, may serve not only to maintain the metal in molten condition, but also to cause agitation thereof by being directed upon the surface of the molten metal.

By my improved process an extra strong ductile union is formed between the parts 110 united which when placed under stress will always result in a shearing through of the more ductile copper casting.

The order in which the copper rod and copper article are melted is not material since the copper rod containing the silicon can be first melted to form a portion of the bath and then the copper article can be melted into this bath. When it is not desired to unite a copper article to a ferrous article but merely to unite only a small amount of copper, all of which is to be melted, to the ferrous article, it will be understood that it is only necessary to melt the copper in the presence of the proper amount of silicon and maintain the temperature and heating conditions substantially as disclosed hereinabove until the metals unite.

In case it is desired to unite two articles

of iron or steel by a copper alloy between the same, the articles are placed in position with their surfaces to be united slightly spaced apart and copper silicon rod, or copper to which silicon is continuously added is melted into said space and maintained at such a temperature and under such conditions that the copper will unite with the iron.

10 By means of this process copper can be united to steel or two articles of steel can be united by a body of copper alloyed to each, without melting an appreciable amount of the iron, or, so far as I am 15 able to determine disadvantageously changing the physical character thereof.

This process is available for use for many industrial purposes, for example, in the welding of copper bonds to steel rails, in 20 welding copper terminals to iron rods and for numerous other purposes.

It is believed that the process is also applicable to welding copper to other metals but specific application of this process to 25 such other metals will be set forth in separate applications for patent.

It will be understood that I do not limit myself to silicon as a reagent for use in my process, as other substitutes and equivalents are known or may be found, for example, manganese or aluminum may be used in connection with the welding of copper to steel.

35 It is also recognized that changes and modifications within the knowledge and skill of those skilled in the art may be employed without departing from the spirit of my invention, the scope of which is defined by what is claimed.

40 Furthermore it is to be understood that the particular forms of apparatus shown and described, and the particular procedure set forth, are presented for purposes of explanation and illustration and that various 45 modifications of said apparatus and procedure can be made without departing from my invention as defined in the appended claims.

What I claim is:

50 1. The process of uniting metals, one of which has an oxidized surface, which comprises melting one of the said metals in contact with the other metal having an oxidized surface and in the presence of a reagent capable of removing the oxide from the surface of said other metal, and continuing the application of heat until the reagent removes the oxide from the surface of said other metal, and the two metals unite.

55 2. The process of uniting the metal of one article to another metallic article having an oxidized surface, which comprises melting a portion of the metal of said first article into contact with the other said article and 60 in the presence of an oxide removing sub-

stance, and heating the molten metal until substantially all oxide has been removed from the surface of said other metal which is in contact with the said molten metal and until the metals unite throughout their contacting surfaces and are joined together.

65 3. The process of uniting a non-ferrous metal to a ferrous metal having an oxidized surface which comprises bringing the non-ferrous metal in molten form into contact with the said ferrous metal in the presence of an oxide removing substance and heating the metals until the said substance has removed the oxide from the surfaces of the ferrous metal in contact with the non-ferrous metal and until the non-ferrous metal has penetrated into and united with the said ferrous metal.

70 4. The process of uniting a non-ferrous metal to a ferrous metal having an oxidized surface which comprises bringing the non-ferrous metal in molten condition into contact with the ferrous metal, and removing in the form of a slag the oxide from the surface of the ferrous metal thereby permitting the metals to unite throughout substantially non-oxidized contacting surfaces.

75 5. The process of uniting non-ferrous and ferrous metals which comprises bringing molten non-ferrous metal into contact with the ferrous metal having an oxidized surface in the presence of a reagent capable of reacting with metallic oxides to form a slag, heating the molten non-ferrous metal without melting a substantial amount of the ferrous metal until a molten slag is formed on the non-ferrous metal and an alloy film is formed throughout the non-oxidized contacting surfaces of the said metals.

80 6. The process of uniting non-ferrous and ferrous metals which comprises bringing molten non-ferrous metal into contact with the ferrous metal having an oxidized surface in the presence of a reagent capable of reacting with metallic oxides to form a slag, heating the molten non-ferrous metal by means of an electric arc directed thereon without melting a substantial amount of the ferrous metal until a molten slag is formed on the non-ferrous metal and an alloy film is formed throughout the non-oxidized contacting surfaces of the said metals.

85 7. The process of uniting copper to a ferrous metal which comprises bringing the molten copper containing silicon into contact with the ferrous metal having an oxidized surface, heating the copper without melting a substantial amount of the ferrous metal until a slag containing silicon is formed on the molten copper and an alloy film is formed throughout substantially the deoxidized contacting surfaces of the said metals.

90 8. The process of uniting non-ferrous

- metal to a ferrous metal which comprises bringing the molten non-ferrous metal into contact with the ferrous metal having an oxidized surface in the presence of a substance capable of reacting with metallic oxides on the ferrous metal to form a slag, heating the molten non-ferrous metal without melting a substantial amount of the ferrous metal until the reagent forms a slag with the oxides on the ferrous metal and until the non-ferrous metal wets the ferrous metal substantially throughout the deoxidized contacting surfaces. 14. The process of uniting metals having oxidized surfaces which comprises bringing into contact with the said surfaces molten metal containing an oxide removing substance, applying heat under suitable conditions of time and temperature to cause the said oxide removing substance to react with the said oxidized surfaces and to deoxidize said metallic surfaces beneath the surface of said molten metal, and to cause said metals to unite in the absence of gases and oxides. 70
9. The process of uniting copper to steel which comprises bringing the copper in molten condition into contact with the steel having an oxidized surface in the presence of silicon, heating the copper without melting a substantial amount of the steel until a molten slag forms on the copper and until the molten copper wets the steel substantially throughout the non-oxidized contacting surfaces. 15. The process of uniting metals which comprises bringing the metals into contact with each other, melting one of the metals, disseminating throughout the molten metal a reagent capable of reacting with metallic oxides to remove the same, causing the reagent to remove oxides from the molten metal and any oxide from the surfaces of contact of the metals, and causing an alloy film to unite the metals throughout their contacting surfaces. 80
10. The process of uniting copper to steel which comprises bringing molten copper containing silicon into contact with the steel having an oxidized surface and applying heat directly to the molten copper until substantially all oxide has been removed from the surface of the steel which is in contact with the copper and until the copper has united with the steel throughout their contacting surfaces. 16. The process of uniting metals which comprises bringing the metals into contact with each other, melting one of the metals and disseminating throughout the molten metal a reagent capable of reacting with metallic oxides to remove the same, heating the molten metal by an electric arc thus causing the reagent to react with the oxides from the molten metal and from the surfaces of contact of the metals and remove the same, and thereby permitting an alloy film to unite the metals throughout their contacting surfaces. 90
11. The process of uniting a copper article to a steel article which comprises melting a portion of the said copper article into contact with the steel article having an oxidized surface in the presence of silicon and applying heat directly to the molten copper until any oxide on the steel article in contact with the molten copper has been removed and until the molten copper has penetrated slightly into the steel article. 17. The process of uniting metals which comprises bringing the metals into contact with each other, melting one of the metals, disseminating throughout the molten metal a reagent capable of reacting with metallic oxides to remove the same, heating the reagent by means of an electric arc directed on the molten metal to remove oxides from the molten metal and any oxide from the surfaces of contact of the metals, and causing an alloy film to unite the metals throughout their contacting surfaces. 100
12. The process of uniting a copper article to a steel article which comprises melting a portion of the said copper article into contact with the steel article having an oxidized surface in the presence of silicon and applying heat directly to the molten copper by means of an electric arc until any oxide on the steel article in contact with the molten copper has been removed and until the molten copper has penetrated slightly into the steel article. 18. The process of uniting copper and steel which comprises bringing molten copper containing silicon into contact with steel having an oxidized surface, heating the copper to a temperature above the melting point thereof and maintaining the temperature until the oxides are removed from the copper and from the surface of the steel and the metals unite with each other substantially without any intervening oxide or non-metallic substances throughout their contacting surfaces. 110
13. The process of uniting metals having oxidized surfaces which comprises bringing into contact with the said surfaces molten metal containing an oxide removing substance, applying heat under suitable conditions of time and temperature to cause the said oxide removing substance to react with the said oxidized surfaces and to expose deoxidized metallic surfaces to the molten metal and cause it to unite therewith in the absence of gases and oxides. 19. The process of uniting copper and steel which comprises bringing molten copper containing silicon into contact with steel having an oxidized surface, heating the copper by means of an electric arc directed thereon to a temperature above the melting

point thereof and maintaining the temperature until the oxides are removed from the copper and from the surface of the steel and the metals unite with each other substantially without any intervening oxide or non-metallic substances throughout their contacting surfaces.

20. The process of uniting copper to steel which comprises melting the copper adjacent to the steel and heating the copper above its melting point in the presence of a deoxidizing reagent by directing a flame upon the copper without directing the flame upon the steel and maintaining the copper above its melting point without melting a substantial amount of the steel until the copper wets the steel and a substantially clean, non-porous alloy junction is formed between the copper and the steel throughout their contacting surfaces.

21. The process of uniting copper to steel which comprises melting the copper adjacent to the steel and heating the copper above its melting point in the presence of a deoxidizing reagent by directing an electric arc upon the copper without directing the arc upon the steel and maintaining the copper above its melting point without melting a substantial amount of the steel until the copper wets the steel and a substantially clean, non-porous alloy junction is formed between the copper and the steel throughout their contacting surfaces.

22. The process of uniting copper to steel which comprises striking an arc with a copper electrode, melting copper by said arc in the presence of a deoxidizing reagent into contact with the steel without directing the arc upon the steel and maintaining the molten copper above its melting point until the copper wets the steel and a substantially clean, non-porous alloy junction is formed between the copper and the steel throughout their contacting surfaces.

23. The process of uniting copper and steel having an oxidized surface which consists in successively melting separate portions of copper adjacent to the steel without melting the steel, and supplying silicon to such successively melted portions in quantities sufficient to reduce or remove any oxide from the surface of the steel with which the molten copper contacts, and maintaining the copper at a temperature above its melting point and below the melting point of the steel until any oxide is removed from the surface of the steel in contact with the molten copper and until an alloy film is formed throughout their contacting surfaces.

24. The process of uniting metals which comprises bringing two metals having oxidized surfaces in the solid state substantially into surface contact with each other, melting one of the said metals, causing a reagent to

remove oxides from the molten metal and any oxide from the surfaces of contact of the metals so as to permit the metals in contact beneath the surface of the molten metal to unite, and maintaining a heating flame upon the molten metal until the reaction of the reagent substantially is completed and the metals have united throughout substantially deoxidized contacting surfaces.

25. The process of uniting metals which comprises bringing two metals having oxidized surfaces in the solid state substantially into surface contact with each other, melting one of the said metals by the application thereto of heat from an electric arc, disseminating throughout the molten metal a reagent capable of reacting with metallic oxides to remove the same, causing said reagent under influence of the electric arc to remove oxides from the molten metal and any oxide from the contacting surfaces of the metals so as to permit the thus cleaned metals in contact beneath the surface of the molten metal to unite, and maintaining the electric arc upon the molten metal until the reaction of the reagent substantially is completed and the metals have united throughout substantially deoxidized contacting surfaces.

26. The process of uniting metals which comprises bringing two metals having oxidized surfaces in the solid state substantially into surface contact with each other, melting one of said metals by the application of heat from an electric arc, one electrode of which is constituted by one of said metals and the other electrode of which is constituted by a rod of the same metal having alloyed therewith or carried thereby a reagent capable of reacting with metallic oxides to remove the same, causing said reagent under the influence of said electric arc to remove oxides from the molten metal and from the contacting surfaces of the metals so as to permit the thus cleaned metals in contact beneath the surface of the molten metal to unite, and maintaining the electric arc upon the molten metal until the reaction of the reagent substantially is completed and the metals have united throughout substantially deoxidized contacting surfaces.

27. The process of uniting copper and iron which consists in adding silicon to the copper and causing the same to be disseminated throughout the copper, then melting the copper into contact with iron, causing the silicon to react with any oxide on the surface of the iron in contact with the molten copper and maintaining said copper molten until an alloy junction is formed throughout the copper and the iron.

In testimony whereof, I hereunto affix my signature.

JOHN B. AUSTIN.